

## UNITED STATES PATENT OFFICE.

WILBUR L. WRIGHT, OF FULTON, NEW YORK.

## ART OF RENDERING PAPER AND OTHER FIBROUS MATERIAL IMPERVIOUS TO GREASE.

No Drawing.

Application filed May 12, 1920. Serial No. 380,752.

*To all whom it may concern:*

Be it known that I, WILBUR L. WRIGHT, a citizen of the United States of America, and resident of Fulton, county of Oswego, State of New York, have invented certain new and useful Improvements in and Relating to the Art of Rendering Paper and Other Fibrous Material Impervious to Grease, of which the following is a specification.

10 This invention relates to the art of rendering paper and other fibrous material impervious to grease; and the objects and nature of the invention will be readily understood by those skilled in the art in 15 the light of the following explanation of what I now believe to be the preferred expression and embodiment of the invention.

The object of the invention is to provide paper or other fibrous material either impregnated with or having a coating of improved material that establishes a barrier against the passage of grease, material that is not soluble in grease, and that can be applied to the paper or other material, either 25 hot or cold, and to provide an improved composition for such purpose.

With these and other objects in view, the invention consists in a composition, or in paper or other fibrous material impregnated 30 with or having a coating of such composition, where such composition embodies casein.

The basis of the composition of my invention is characterized by a body, adhesive, or 35 gelatinous solution composed of a casein solution, whether or not other ingredients are included to control the flexibility and hardness of the coating formed by the composition, or to render the same waterproof, 40 or to attain other qualities not inherent in the casein solution.

The casein solution can be formed by various methods well known to those skilled in the art.

45 For instance, I can use a solvent consisting of water and ammonia by which the casein is dissolved in the presence of heat.

As an example, a grease proofing composition embodying my invention can be composed of, say two hundred parts, more or less

of casein; ammonia, ten parts more or less; water one thousand parts more or less; and glycerine (or some other ingredient to maintain the desired flexibility of the coating formed by the composition) ten parts 55 more or less.

This composition can be formed by soaking the casein in the ammonia diluted by about one half the proportion of water. 60 After the casein has soaked for several hours, add the other half of the water proportion and the glycerine and maintain the mixture at a suitable temperature (say about 175° Fah.) and stir until the casein has dissolved. Before using the composition, I usually filter or decant the same to remove any possibility of remaining undissolved portions of casein.

This composition can be applied to the paper or other material, either hot or cold. 70 This is a material advantage in practice. The composition is usually applied to form a coating on paper for use in the arts and is of particular advantage for coating the inner surfaces of paper containers for 75 grease-like products, particularly food products such as lards and artificial lards and the like.

The casein is a pure clean product and has no deleterious action on food products.

The proportions stated can be greatly varied and various other ingredients can be added to the composition and other ingredients can be substituted for glycerine, all without departing from my invention, i. e. 85 utilizing casein to form the body or basis of the composition.

What I claim is:—

1. A paper container for food products 90 internally grease-proofed by a composition of casein containing a small percentage of flexibility ingredient.

2. A paper material container for food products, grease-proofed by a layer of 95 casein composition.

3. A paper material container having an internal grease-proofing layer composed of a composition of dissolved casein rendered flexible by glycerine.

WILBUR L. WRIGHT.